

# United States Patent

[11] 3,615,522

[72] Inventors **Reiichi Ohi;**  
**Haruhiko Iwano; Tadao Shishido; Isao**  
**Shimamura, all of Kanagawa, Japan**  
[21] Appl. No. **842,011**  
[22] Filed **July 15, 1969**  
[45] Patented **Oct. 26, 1971**  
[73] Assignee **Fuji Photo Film Co., Ltd.**  
**Kanagawa, Japan**  
[32] Priority **July 15, 1968**  
[33] **Japan**  
[31] **43/49818**

[54] **PROCESS FOR DEVELOPMENT OF MULTILAYER COLOR PHOTOGRAPHIC MATERIALS**  
17 Claims, No Drawings  
[52] U.S. Cl. .... **96/66 R,**  
96/22  
[51] Int. Cl. .... **G03c 5/50,**  
**G03c 5/52, G03c 5/30**

[50] **Field of Search**..... 96/59, 66.3,  
22, 55

[56] **References Cited**  
UNITED STATES PATENTS  
3,017,270 1/1962 Tregillus et al. .... 96/29

*Primary Examiner*—Norman G. Torchin  
*Assistant Examiner*—Alfonso T. Suro Pico  
*Attorney*—Sughrue, Rothwell, Mion, Zinn & Macpeak

**ABSTRACT:** Method of processing a silver halide multilayer color photographic material which comprises the incorporation of a mercaptotriazole compound into one of the processing solutions. Such incorporation causes selective inhibition of the development of the uppermost emulsion layer, resulting in a developed material possessing improved, balanced contrast.

**PROCESS FOR DEVELOPMENT OF MULTILAYER COLOR PHOTOGRAPHIC MATERIALS**

**BACKGROUND OF THE INVENTION**

**1. Field of the Invention**

This invention relates to a method of developing a color photographic material, in particular, by the use of a compound available in a high temperature rapid processing.

**2. Description of the Prior Art**

Multilayer color photographic material generally has at least three kinds of silver halide emulsion layers, each differing in color sensitivity, superimposed on a support, for example, a blue-sensitive emulsion as uppermost layer, yellow filter layer, green-sensitive emulsion layer and red-sensitive emulsion layer.

Of late, the method of developing color-sensitive materials has undergone a change, particularly in that the developing temperature has been raised to shorten the developing time. This is ordinarily called the "high temperature rapid-processing method." One of the difficulties encountered in the development of multilayer materials, especially when the development is carried out at high temperatures, is the overdevelopment of the uppermost emulsion layer before the lower emulsion layers are completely developed. The overdevelopment, which is caused primarily by the excessive concentration of the developer in the uppermost layer, results in disproportionate image density in that layer as compared to the remaining layers.

To overcome this disadvantage, it is known to add a development inhibitor, which inhibits the overdevelopment of the uppermost layer, to the processing solution, but the addition of commonly used development inhibitors, such as for example 6-nitroisoindazole, is not always suitable for this purpose since the effect extends to the lowermost layer as well as the uppermost layer.

In order to avoid this disadvantage, it is known to add an acylaminophenyl mercaptotetrazole compound to a development solution (cf. U.S. Pat. No. 3,295,967), so that the development of only the uppermost layer is selectively inhibited and development throughout all of the layers is well balanced. However, the difficulty of this method is that the mercaptotetrazole compound disclosed in this patent is synthesized from thiophosgene which is generally hard to obtain.

**SUMMARY OF THE INVENTION**

It is the principal object of the invention to provide a method using a mercaptotriazole compound as a development inhibitor for the uppermost layer in the high temperature rapid-processing treatment of a silver halide multilayer color photographic material.

We have discovered that selective inhibition can be achieved by adding a mercaptotriazole compound, which can readily be synthesized, to a preprocessing solution or to a developing solution.

**DETAILED DESCRIPTION OF THE INVENTION**

In the high temperature rapid-processing method of this invention, a mercaptotriazole compound is added to a developing solution or to a preprocessing solution prior to development, whereby to suppress selectively the progress of development of only the uppermost layer of multilayer color-sensitive material, to inhibit overdevelopment of the uppermost layer, thereby improving the color balance and image quality obtained.

A particular advantage of the present invention lies in the ability to process at a temperature of from 30° to 70° C. when using a compound of the invention.

The above preprocessing solution is usually a prehardening bath consisting of an aqueous solution containing one or more aldehydes having the ability to harden gelatin, a component of the photographic emulsion. Examples of these are formaldehyde, glyoxal, succinaldehyde and glutaraldehyde. This

solution also would normally contain a salt such as sodium sulfate, a buffering agent such as borax, acetic acid, sodium acetate, sodium hydroxide, sodium carbonate, sulfuric acid or boric acid and a fog inhibitor such as an alkali metal halide.

5 The first developing solution of a color reversal film is an aqueous solution containing one or more developing agents such as hydroquinone, 1-phenyl-3-pyrazolidone or N-methyl-p-aminophenol, to which may be added a salt such as sodium sulfate, a buffering agent such as borax, boric acid, sodium hydroxide or sodium carbonate and a fog inhibitor such as an alkali metal halide.

10 The color-developing solution of a color negative film or color paper is an alkaline aqueous solution containing one or more p-phenylenediamine derivatives such as N,N-diethyl-p-phenylenediamine sulfite, N,N-diethyl-3-methyl-p-phenylenediamine hydrochloride, 4-amino-3-methyl-N-ethyl-N-methanesulfonamideethylaniline sulfate, 4-amino-3-methyl-N-ethyl-N-hydroxyethylaniline sulfate or N-ethyl-N-hydroxyethyl-p-phenylenediamine sulfate, to which may ordinarily be added a salt such as sodium sulfate, a buffering agent such as sodium hydroxide, sodium carbonate or sodium phosphate and the usual fog inhibitor such as an alkali metal halide.

15 The object of the invention can be achieved by adding, to one or more of the above processing solutions, a mercaptotriazole compound represented by the following formula



20 35 in which R<sub>1</sub> and R<sub>2</sub> may be the same or different and each represents hydrogen, alkyl such as methyl, ethyl, propyl, butyl, amyl, hexyl, heptyl, octyl, nonyl, decyl, undecyl, dodecyl, tetradecyl, hexadecyl, octadecyl, eicosyl and the like, and



40 45 (wherein R<sub>3</sub> represents hydrogen, amino or



50 50 wherein R<sub>4</sub> represents alkyl such as methyl, ethyl, propyl, butyl, amyl, hexyl, heptyl, octyl, nonyl, decyl, undecyl, dodecyl, tetradecyl, hexadecyl, octadecyl, eicosyl and the like).

55 The compounds of the present invention are used in connection with the color processing of multilayer photographic materials well known in the art. Such materials generally comprise a support of cellulose ester, paper or other suitable base having coated thereon a red-sensitive emulsion layer containing a cyan-forming coupler, a green-sensitive emulsion layer

60 containing a magenta-forming coupler and a blue-sensitive emulsion layer containing a yellow-forming coupler. The couplers may be incorporated in any manner known in the art. The compounds of the present invention are, however, not limited in their use to the above-described multilayer material.

65 The photographic material may contain fewer or more sensitive emulsion layers and may also contain conventional filter layers, inter layers, subbing layers, backing layers and overcoating layers. Further, for example, one or more of the emulsion layers may be free of incorporated couplers, the coupler or couplers for these layers being contained in the color developing solution.

70 75 According to the present invention, the mercaptotriazole compound is applied during processing to the image-exposed multilayer color photographic material so that this compound is present in the top silver emulsion layer (but not in the mid-

dle or bottom layers) during the negative development step of the color process.

The following are typical examples of the compounds used in the method of this invention. However, the compounds of this invention are not limited only to these examples, which are presented for purposes of illustration.

Compound 1.—3-mercaptop-4-phenyl-1, 2, 4-triazole, M.P. 172°C.



Compound 2.—3-mercaptop-5-methyl-4-phenyl-1, 2, 4-triazole, M.P. 224°C.



Compound 3.—5-ethyl-3-mercaptop-4-phenyl-1, 2, 4-triazole, M.P. 177°C.



Compound 4.—3-mercaptop-5-pentyl-4-phenyl-1, 2, 4-triazole, M.P. 137°C.



Compound 5.—4, 5-diphenyl-3-mercaptop-1, 2, 4-triazole, M.P. 280°C.



Compound 6.—3-mercaptop-4-phenyl-5-undecyl-1, 2, 4-triazole, M.P. 103°C.



Compound 7.—4, 5-diethyl-3-mercaptop-1, 2, 4-triazole, M.P. 148°C.



Compound 8.—4-ethyl-3-mercaptop-5-pentyl-1, 2, 4-triazole, M.P. 86°C.



Compound 9.—4-ethyl-3-mercaptop-5-phenyl-1, 2, 4-triazole, M.P. 145°C.



Compound 10.—5-p-aminophenyl-4-ethyl-3-mercaptop-1, 2, 4-triazole, M.P. 245°C.



Compound 11.—5-p-acetoamidophenyl-4-ethyl-3-mercaptop-1, 2, 4-triazole, M.P. 252°C.



Compound 12.—5-p-caproamidophenyl-4-ethyl-3-mercaptop-1, 2, 4-triazole, M.P. 216°C.



Compound 13.—4-ethyl-5-p-lauroamidophenyl-3-mercaptop-1, 2, 4-triazole, M.P. 155°C.



## EXAMPLE VI

The above compounds can easily be synthesized by reaction of 4-substituted thiosemicarbazide and an acid anhydride (cf. British Pat. No. 766,380) or acid chloride (cf. Ohta and Toshima, "Nippon Yakugaku Zasshi (Japan Pharmacology Journal)" Vol. 72, p. 376 (1952)), or by the reaction of a substituted benzoyl hydrazine with a thioisocyanate.

The following are examples of the preparation of selected compounds to be used in the method of this invention.

## EXAMPLE I—5-ethyl-3-mercaptop-4-phenyl-1,2,4-triazole

10 g. of 4-phenylthiosemicarbazide was dissolved in 80 ml. of pyridine and cooled with ice while stirring. 8 g. of propionyl chloride was then gradually added to this solution in drops. After the addition, the mixture was cooled with ice for 1 hour while stirring and then added to ice water and filtered. The resulting crystals were added to 80 ml. of a 10 percent aqueous solution of caustic soda, heated for 2 hours on a water bath, cooled, acidified with hydrochloric acid, filtered and recrystallized from ethanol to obtain 6 g. of the product as needles, melting at 177°C.

## EXAMPLE II—3-mercaptop-5-pentyl-4-phenyl-1,2,4-triazole

10 g. of 4-phenylthiosemicarbazide was dissolved in 80 ml. of pyridine and cooled with ice while stirring. 8 g. of caproyl chloride was then gradually added to this solution in drops. The reaction mixture was then processed as in example I and the resulting crystals recrystallized from ethanol to obtain 7 g. of the product as needles, melting at 136°–137°C.

## EXAMPLE III—4,5-diethyl-3-mercaptop-1,2,4-triazole

9 g. of 4-ethylthiosemicarbazide was dissolved in 50 ml. of pyridine and cooled with ice while stirring. 10 g. of propionyl chloride was then gradually added to this solution in drops. The reaction mixture was then processed as in example I and the resulting crystals recrystallized from water to obtain 6 g. of the product as needles, melting at 148°C.

## EXAMPLE IV—4-ethyl-3-mercaptop-5-phenyl-1,2,4-triazole

9 g. of 4-ethylthiosemicarbazide was dissolved in 50 ml. of pyridine and cooled with ice while stirring. 15 g. of benzoyl chloride was then gradually added to this solution in drops. The reaction mixture was then processed as in example I and the resulting crystals recrystallized from a mixed solvent of water and ethanol to obtain 9 g. of the product as needles, melting at 145°C.

## EXAMPLE V—5-p-aminophenyl-4-ethyl-3-mercaptop-1,2,4-triazole

12.5 g. of p-acetamidobenzoylhydrazine was dissolved in 100 ml. of ethanol. 10 ml. of ethylthioisocyanate was then added and the mixture refluxed for 2 hours. After cooling, the resulting crystals were filtered, added to 20 ml. of 10 percent aqueous solution of caustic soda, refluxed for 2 hours on a water bath, cooled and acidified with hydrochloric acid and filtered. The resulting crystals were recrystallized from ethanol to obtain 9 g. of the product as needles, melting at 244°–245°C.

The compounds of this invention may be employed in a wide range of concentrations, i.e., from about  $1 \times 10^{16}$  mol/liter to about  $1 \times 10^{12}$  mol/liter. The optimum concentration depends upon a number of factors, for example, the particular compound used, composition of the treating solution, the activity of the developing solution, the treating temperature, the particular characteristics of the multilayer color-sensitive material, etc. The optimum concentration to be employed in any particular circumstance can be readily determined by methods well known in the art.

The following examples are given in order to illustrate the invention in detail without limiting the same.

A multilayer color film prepared by successively applying to a cellulose acetate support a gelatino iodoform emulsion sensitive to red light, a gelatino iodoform emulsion sensitive to green light, a yellow filter layer containing colloidal silver capable of absorbing blue light, and a gelatino iodoform emulsion sensitive to blue light, was exposed on a sensitometer and then subjected to the following processes:

|    | Processing steps                                       | Temperature (°C.) | Time               |
|----|--------------------------------------------------------|-------------------|--------------------|
| 5  | Prehardening                                           | 40                | 30 sec.            |
| 10 | Water washing                                          | 40                | 30 sec.            |
| 15 | First developing                                       | 40                | 75 sec.            |
| 20 | Water washing                                          | 40                | 30 sec.            |
| 25 | Reversal exposure (red light)<br>from back of film     | 200 CMS           |                    |
| 30 | Cyan color developing                                  | 40                | 3 min.             |
| 35 | Water washing                                          | 40                | 30 sec.            |
| 40 | Reversal exposure (blue light)<br>from surface of film | 200 CMS           |                    |
| 45 | Yellow color developing                                | 40                | 1 min.,<br>30 sec. |
| 50 | Water washing                                          | 40                | 30 sec.            |
| 55 | Second black-and-white<br>developing                   | 40                | 15 sec.            |
| 60 | Magenta color developing                               | 40                | 2 min.             |
| 65 | Water washing                                          | 40                | 1 min.             |
| 70 | Bleaching                                              | 40                | 1 min.             |
| 75 | Fixing                                                 | 40                | 1 min.             |
| 80 | Water washing                                          | 40                | 1 min.             |

The processing solutions employed in the above series of processing steps had the following compositions:

|    |                                          |           |
|----|------------------------------------------|-----------|
| 35 | Prehardening solution                    |           |
| 40 | sodium hexametaphosphate                 | 1.0 g.    |
| 45 | sodium bisulfite                         | 5.0 g.    |
| 50 | sodium pyrophosphate                     | 15.0 g.   |
| 55 | sodium sulfate                           | 150.0 g.  |
| 60 | potassium bromide                        | 2.0 g.    |
| 65 | sodium hydroxide                         | 0.1 g.    |
| 70 | formalin (37%)                           | 15.0 ml.  |
| 75 | water to make                            | 1,000 ml. |
| 35 | First developing solution                |           |
| 40 | N-methyl-p-aminophenol                   | 5.0 g.    |
| 45 | sodium sulfite                           | 70.0 g.   |
| 50 | hydroquinone                             | 2.0 g.    |
| 55 | sodium carbonate monohydrate             | 41.0 g.   |
| 60 | potassium bromide                        | 4.0 g.    |
| 65 | potassium thiocyanate                    | 1.6 g.    |
| 70 | potassium iodide (0.1% aqueous solution) | 10.0 ml.  |
| 75 | water to make                            | 1,000 ml. |
| 35 | Cyan color developing solution           |           |
| 40 | potassium bromide                        | 3.0 g.    |
| 45 | 6-nitrobenzimidazole                     | 0.03 g.   |
| 50 | potassium iodide (0.1% aqueous solution) | 10.0 ml.  |
| 55 | sodium sulfite                           | 10.0 g.   |
| 60 | sodium sulfate                           | 60.0 g.   |
| 65 | potassium thiocyanate                    | 1.0 g.    |
| 70 | 4-amino-3-methyl-N-ethyl-N-              |           |
| 75 | hydroxyethylaniline sulfate              | 2.5 g.    |
| 35 | sodium hydroxide                         | 3.0 g.    |
| 40 | 1,5-dihydroxy-2,6-dibromonaphthalene     | 2.0 g.    |
| 45 | monobenzyl-p-aminophenol                 | 0.4 g.    |
| 50 | p-aminophenol hydrochloride              | 0.1 g.    |
| 55 | water to make                            | 1,000 ml. |
| 35 | Yellow color developing solution         |           |
| 40 | sodium sulfite                           | 10.0 g.   |
| 45 | potassium bromide                        | 0.5 g.    |
| 50 | potassium iodide (0.1% aqueous solution) | 25.0 ml.  |
| 55 | 6-nitrobenzimidazole                     | 0.1 g.    |
| 60 | sodium sulfate                           | 60.0 g.   |
| 65 | N,N-diethyl-p-phenylenediamine sulfite   | 2.5 g.    |
| 70 | sodium hydroxide                         | 2.5 g.    |
| 75 | W-benzoyl-4-(p-toluenesulfonamide)       | 1.8 g.    |
| 35 | acetanilide                              |           |
| 40 | water to make                            | 1,000 ml. |
| 35 | Magenta color developing solution        |           |

|                                                       |           |
|-------------------------------------------------------|-----------|
| sodium sulfite                                        | 5.0 g.    |
| potassium bromide                                     | 1.0 g.    |
| potassium thiocyanate                                 | 1.0 g.    |
| sodium sulfate                                        | 60.0 g.   |
| N,N-diethyl-3-methyl-p-phenylenediamine hydrochloride | 2.5 g.    |
| sodium hydroxide                                      | 2.0 g.    |
| 1-phenyl-3-(m-nitrobenzoylamino)-5-pyrazolone         | 1.4 g.    |
| ethylenediamine                                       | 8.0 ml.   |
| water to make                                         | 1,000 ml. |
| Bleaching solution                                    |           |
| potassium ferricyanide                                | 100 g.    |
| potassium bromide                                     | 30.0 g.   |
| water to make                                         | 1,000 ml. |
| Fixing solution                                       |           |
| sodium thiosulfate                                    | 150 g.    |
| sodium sulfite                                        | 10 g.     |
| water to make                                         | 1,000 ml. |

In the above color reversal developing treatment, a compound of the invention was added to the prehardening solution as tabulated below.

| Test No. | Additive to prehardening                     | Addition amount (mol/liter) |
|----------|----------------------------------------------|-----------------------------|
| 6a       | no additive                                  |                             |
| 6b       | 5-ethyl-3-mercaptop-4-phenyl-1,2,4-triazole  | $1 \times 10^{-4}$          |
| 6c       | 3-mercaptop-5-pentyl-4-phenyl-1,2,4-triazole | $1 \times 10^{-4}$          |
| 6d       | 4-ethyl-3-mercaptop-5-phenyl-1,2,4-triazole  | $1 \times 10^{-4}$          |
| 6e       | 4,5-diethyl-3-mercaptop-1,2,4-triazole       | $1 \times 10^{-4}$          |

The results obtained are shown in the following table. The photographic characteristics are represented by the blue density (DBmax) and the red density (DRmax) in maximum density areas. The blue density is the density of the yellow-dye image in the uppermost blue-sensitive emulsion layer and the red density is the density of the cyan-dye image in the lowermost red-sensitive emulsion layer. It is desired for good color reproduction that both values are large and approximately equal each other.

| Test No. | Blue density (DBmax) | Red density (DRmax) |
|----------|----------------------|---------------------|
| 6a       | 2.3                  | 3.5                 |
| 6b       | 3.6                  | 3.6                 |
| 6c       | 3.2                  | 3.6                 |
| 6d       | 3.2                  | 3.5                 |
| 6e       | 3.4                  | 3.5                 |

It is evident from this table that addition of the compounds of the present invention results in a further increase of the blue density without lowering the red density in any case.

### EXAMPLE VII

Following the processing steps of example I, but adding the compounds of the invention to the first developing solution instead of the prehardening bath, the following results were obtained:

| Test No. | Additive to first developing                 | Addition amount (mol/liter) |
|----------|----------------------------------------------|-----------------------------|
| 7a       | no additive                                  |                             |
| 7b       | 5-ethyl-3-mercaptop-4-phenyl-1,2,4-triazole  | $5 \times 10^{-4}$          |
| 7c       | 3-mercaptop-5-pentyl-4-phenyl-1,2,4-triazole | $5 \times 10^{-4}$          |
| 7d       | 4-ethyl-3-mercaptop-5-phenyl-1,2,4-triazole  | $5 \times 10^{-4}$          |
| 7e       | 4,5-diethyl-3-mercaptop-1,2,4-triazole       | $5 \times 10^{-4}$          |

As in example VI, the photographic characteristic values resulting from the developing are shown as the blue density (DBmax) and red density (DRmax) in the following table.

| Test No. | Blue density (DBmax) | Red density (DRmax) |
|----------|----------------------|---------------------|
| 7a       | 2.3                  | 3.5                 |
| 7b       | 3.9                  | 3.6                 |
| 7c       | 3.7                  | 3.8                 |
| 7d       | 3.6                  | 3.5                 |
| 7e       | 3.7                  |                     |

It is evident from this table that addition of the compounds of the present invention results in a further increase of the blue density without lowering the red density in any case.

### EXAMPLE VIII

A multilayer reversal color film having silver halide emulsion layers containing a color coupler and having three different sensitivity regions was exposed by a sensitometer and subjected to the following processing steps.

| Test No. | Processing steps | Temperature (°C.) | Time (min.) |
|----------|------------------|-------------------|-------------|
| 25       | First developing | 37                | 3           |
|          | First stopping   | 37                | 1/2         |
|          | Water washing    | 37                | 1           |
| 30       | Color developing | 37                | 3 1/2       |
|          | Second stopping  | 37                | 1/2         |
|          | Water washing    | 37                | 1           |
|          | Bleaching        | 37                | 1 1/2       |
|          | Fixing           | 37                | 1           |
|          | Water washing    | 37                | 1           |

The compositions of the processing solutions were as follows:

| Test No. | First developing solution                                                                                                                                                                                                                                                                                                                                               |
|----------|-------------------------------------------------------------------------------------------------------------------------------------------------------------------------------------------------------------------------------------------------------------------------------------------------------------------------------------------------------------------------|
| 40       | sodium hexametaphosphate 1.0 g.<br>1-phenyl-3-pyrazolidone 0.3 g.<br>sodium sulfite 50.0 g.<br>hydroquinone 6.0 g.<br>sodium carbonate monohydrate 35.0 g.<br>potassium bromide 2.0 g.<br>potassium thiocyanate 1.0 g.<br>potassium iodide (0.1% aqueous solution) 10 ml.<br>water to make 1,000 ml.                                                                    |
| 45       | First stopping solution and second stopping solution                                                                                                                                                                                                                                                                                                                    |
| 50       | acetic acid 25 ml.<br>sodium acetate 3 g.<br>water to make 1,000 ml.                                                                                                                                                                                                                                                                                                    |
| 55       | Color developing solution                                                                                                                                                                                                                                                                                                                                               |
|          | sodium hexametaphosphate 1.0 g.<br>benzyl alcohol 6.0 ml.<br>sodium sulfite 5.0 g.<br>sodium phosphate, tribasic 40.0 g.<br>potassium bromide 0.2 g.<br>potassium iodide (0.1% aqueous solution) 10.0 ml.<br>sodium hydroxide 3.5 g.<br>4-amino-3-methyl-N-ethyl-N-methanesulfonamideethylaniline sulfate 10.0 g.<br>ethylenediamine 8.0 ml.<br>water to make 1,000 ml. |

| Test No. | Additive to first developing                 | Addition amount (mol/liter) | First developing solution                                                                                                                                                                                                                                                                                                                                                                                                               |
|----------|----------------------------------------------|-----------------------------|-----------------------------------------------------------------------------------------------------------------------------------------------------------------------------------------------------------------------------------------------------------------------------------------------------------------------------------------------------------------------------------------------------------------------------------------|
| 7a       | no additive                                  |                             | sodium hexametaphosphate 1.0 g.<br>1-phenyl-3-pyrazolidone 0.3 g.<br>sodium sulfite 50.0 g.<br>hydroquinone 6.0 g.<br>sodium carbonate monohydrate 35.0 g.<br>potassium bromide 2.0 g.<br>potassium thiocyanate 1.0 g.<br>potassium iodide (0.1% aqueous solution) 10 ml.<br>sodium hydroxide 3.5 g.<br>4-amino-3-methyl-N-ethyl-N-methanesulfonamideethylaniline sulfate 10.0 g.<br>ethylenediamine 8.0 ml.<br>water to make 1,000 ml. |
| 7b       | 5-ethyl-3-mercaptop-4-phenyl-1,2,4-triazole  | $5 \times 10^{-4}$          |                                                                                                                                                                                                                                                                                                                                                                                                                                         |
| 7c       | 3-mercaptop-5-pentyl-4-phenyl-1,2,4-triazole | $5 \times 10^{-4}$          |                                                                                                                                                                                                                                                                                                                                                                                                                                         |
| 7d       | 4-ethyl-3-mercaptop-5-phenyl-1,2,4-triazole  | $5 \times 10^{-4}$          |                                                                                                                                                                                                                                                                                                                                                                                                                                         |
| 7e       | 4,5-diethyl-3-mercaptop-1,2,4-triazole       | $5 \times 10^{-4}$          |                                                                                                                                                                                                                                                                                                                                                                                                                                         |

In the above internal-type reversal-developing treatment, a compound of the invention was added to the first developing solution. For comparison, a known fog inhibitor, 6-nitroisoindazole, was also used.

| Test No. | Additive to first developing                | Addition amount<br>(mol/liter) |
|----------|---------------------------------------------|--------------------------------|
| 8a       | no additive                                 |                                |
| 8b       | 5-ethyl-3-mercaptop-4-phenyl-1,2,4-triazole | $5 \times 10^{-15}$            |
| 8c       | 4-ethyl-3-mercaptop-5-phenyl-1,2,4-triazole | $5 \times 10^{-15}$            |
| 8d       | 6-nitroisoindazole                          | $5 \times 10^{-15}$            |
| 8e       | 6-nitroisoindazole                          | $5 \times 10^{-14}$            |

The results are shown in the following table in which the photographic characteristic values are given by the blue density (DBmax) and red density (DRmax) on maximum density areas.

| Test No. | Maximum density |             | Reversal sensitivity* |                 |
|----------|-----------------|-------------|-----------------------|-----------------|
|          | blue density    | red density | blue sensitivity      | red sensitivity |
| 8a       | 2.4             | 3.4         | 120                   | 104             |
| 8b       | 3.5             | 3.5         | 100                   | 100             |
| 8c       | 3.3             | 3.5         | 107                   | 102             |
| 8d       | 2.6             | 3.4         | 110                   | 96              |
| 8e       | 3.7             | 3.7         | 68                    | 70              |

\*Reversal sensitivity is the relative sensitivity as compared with the sensitivity resulting from Test No. 8b, which is assigned a value of 100.

It is apparent from this table that the addition of the compounds of this invention results in a sufficiently high-blue density and improved image quality without affecting the sensitivity with good balancing of the blue and red densities. On the other hand, in the test using 6-nitroisoindazole as a known development inhibitor in place of the compounds of this invention for comparison, use of a small amount thereof does not increase the blue density, while use of a large amount thereof results in a very low-reversal sensitivity and does not provide a good image quality, although the blue density is increased. That is, 6-nitroisoindazole inhibits development of both the uppermost layer and the lowermost layer of the emulsion layers, thus lowering the reversal sensitivity. On the other hand, the compounds of the present invention selectively inhibit overdevelopment of the uppermost layer during high temperature processing, thus resulting in a well-balanced development without lowering the reversal sensitivity, as shown in the table.

#### EXAMPLE IX

A multilayer color negative film having silver halide emulsion layers containing a color coupler and having three different sensitivity regions was exposed by a sensitometer and then subjected to the following processing steps.

| Processing steps | Temperature (°C.) | Time (min.) |
|------------------|-------------------|-------------|
| Color developing | 35                | 3           |
| Stopping         | 35                | 1/2         |
| Water washing    | 35                | 1/2         |
| Bleaching        | 35                | 1           |
| Fixing           | 35                | 1 1/2       |
| Water washing    | 35                | 1           |

The compositions of the processing solutions were as follows:

#### Color developing solution

|   |                          |         |
|---|--------------------------|---------|
| 5 | sodium hexametaphosphate | 1.0 g.  |
|   | benzyl alcohol           | 5.0 g.  |
|   | sodium sulfite           | 3.0 g.  |
|   | sodium carbonate         | 41.0 g. |
|   | sodium hydroxide         | 1.0 g.  |

|    |                                                                    |           |
|----|--------------------------------------------------------------------|-----------|
| 10 | 4-amino-3-methyl-N-ethyl-N-methane-sulfonamideethylaniline sulfate | 5.0 g.    |
|    | potassium bromide                                                  | 0.5 g.    |
|    | water to make                                                      | 1,000 ml. |

|    |                |           |
|----|----------------|-----------|
| 15 | acetic acid    | 25 ml.    |
|    | sodium acetate | 3 g.      |
|    | potassium alum | 10 g.     |
|    | water to make  | 1,000 ml. |

|    |                        |           |
|----|------------------------|-----------|
| 20 | potassium ferricyanide | 100 g.    |
|    | potassium bromide      | 20.0 g.   |
|    | water to make          | 1,000 ml. |

|    |                    |           |
|----|--------------------|-----------|
| 25 | sodium thiosulfate | 150 g.    |
|    | sodium sulfite     | 10 g.     |
|    | water to make      | 1,000 ml. |

In the above color-negative-developing treatment, 5-ethyl-3-mercaptop-4-phenyl-1,2,4-triazole (m.p. 177° C.) of the present invention was added to the color developing solution in an amount of  $5 \times 10^{-15}$  mol/liter.

A comparison of the results with those wherein no additive was present showed that the presence of 5-ethyl-3-mercaptop-4-phenyl-1,2,4-triazole (m.p. 177° C.) resulted in the blue-sensitive, green-sensitive and red-sensitive emulsions being developed with improved balance. In other words, excessive development of the blue-sensitive emulsion layer as the uppermost layer is avoided.

What is claimed is:

1. In a method for developing a silver halide multilayer color photographic material selected from the group consisting of a color reversal film, a color negative film and a color paper, the improvement which consists essentially of treating said material with a developing solution consisting essentially of an aqueous solution of at least one developer and a development inhibiting compound represented by the formula:



in which  $\text{R}_1$  and  $\text{R}_2$  are each selected from the group consisting of hydrogen, alkyl and



wherein  $\text{R}_3$  is selected from the group consisting of hydrogen, amino and



wherein  $\text{R}_4$  represents an alkyl group.

3. The method of claim 2 wherein said treatment is conducted at a temperature of from about 30 to about 70° C.

4. The method of claim 2 wherein the concentration of said development-inhibiting compound in said aqueous solution varies from about  $1 \times 10^{-16}$  mole per liter to  $1 \times 10^{-12}$  mole per liter.

5. The method of claim 2 wherein said silver halide multilayer color photographic material is color reversal film and wherein said developer is at least one member selected from the group consisting of hydroquinone, 1-phenyl-3-pyrazolidone and N-methyl-p-aminophenol.

6. The method of claim 2 wherein said silver halide multilayer color photographic material is color negative film or color paper and wherein said developer is at least one p-phenylene-diamine derivative.

7. The method of claim 6 wherein said p-phenylene-diamine derivative is at least one member selected from the group consisting of N,N-diethyl-p-phenylenediamine sulfite, N,N-diethyl-3-methyl-p-phenylenediamine hydrochloride, 4-amino-3-methyl-N-ethyl-N-methanesulfonamideethylaniline methyl-N-ethyl-N-methanesulfonamideethylaniline sulfate, 4-amino-3-methyl-N-ethyl-N-hydroxyethylaniline sulfate or N-ethyl-N-hydroxyethyl-p-phenylenediamine sulfate.

8. The method of claim 1 wherein said alkyl group of R<sub>1</sub>, R<sub>2</sub> and R<sub>4</sub> has from one to 20 carbon atoms.

9. In a method for developing a silver halide multilayer color photographic material, the improvement which consists essentially of treating said material with a preprocessing solution consisting essentially of an aqueous solution of a compound which hardens gelatin and a development-inhibiting compound represented by the formula:



in which R<sub>1</sub> and R<sub>2</sub> are each selected from the group consisting of hydrogen, alkyl and



wherein R<sub>3</sub> is selected from the group consisting of hydrogen, amino and



wherein R<sub>4</sub> represents an alkyl group.

10. The method of claim 9 wherein said development-inhibiting compound is a member selected from the group consisting of 3-mercaptop-4-phenyl-1,2,4-triazole, 3-mercaptop-5-methyl-4-phenyl-1,2,4-triazole, 5-ethyl-3-mercaptop-4-phenyl-1,2,4-triazole, 3-mercaptop-5-pentyl-4-phenyl-1,2,4-triazole, 3-mercaptop-4-phenyl-5-undecyl-1,2,4-triazole, 4,5-diethyl-3-mercaptop-1,2,4-triazole, 4-ethyl-3-mercaptop-5-pentyl-1,2,4-triazole, 4-ethyl-3-mercaptop-5-phenyl-1,2,4-triazole, 5-p-aminophenyl-4-ethyl-3-mercaptop-1,2,4-triazole, 5-p-acetoamidephenyl-4-ethyl-3-mercaptop-1,2,4-triazole, 5-p-caproamidephenyl-4-ethyl-3-mercaptop-1,2,4-triazole and 4-ethyl-5-p-lauroamidophenyl-3-mercaptop-1,2,4-triazole.

11. The method of claim 9 wherein said treatment is conducted at a temperature of from about 30 to about 70°C.

12. The method of claim 9 wherein the concentration of said development-inhibiting compound in said aqueous solution varies from about 1×10<sup>16</sup> mole per liter to about 1×10<sup>12</sup> mole per liter.

13. The method of claim 9 wherein said compound which hardens gelatin is an aldehyde.

14. The method of claim 13 wherein said aldehyde is selected from the group consisting of formaldehyde, glyoxal, succinaldehyde, and glutaraldehyde.

15. The method of claim 9 wherein said aqueous solution further contains a salt, a buffering agent and a fog inhibitor.

16. The method of claim 15 wherein said salt is sodium sulfate, wherein said buffering agent is selected from the group consisting of borax, acetic acid, sodium acetate, sodium hydroxide, sodium carbonate, sulfuric acid and boric acid and wherein said fog inhibitor is an alkali metal halide.

17. The method of claim 9 wherein said alkyl of said R<sub>1</sub>, R<sub>2</sub> and R<sub>4</sub> has from one to 20 carbon atoms.

\* \* \* \* \*